

Aug. 24, 1937.

C. S. GLEZEN

2,090,836

PARTICLE INLAID SURFACE

Filed July 24, 1935



*Carlisle S. Glezen*  
INVENTOR

BY  
*Reydon J. Bushnell*  
ATTORNEY

## UNITED STATES PATENT OFFICE

2,090,836

## PARTICLE INLAID SURFACE

Carlisle S. Glezen, Baldwin, N. Y., assignor to  
 The Safe Tread Company, Inc., New York,  
 N. Y., a corporation of Delaware

Application July 24, 1935, Serial No. 32,840

5 Claims. (Cl. 22—202)

This invention relates to methods for the manufacture of cast metal articles wherein some of the surfaces of the finished article are inlaid with particles, etc., such as abrasive particles, etc., affixed by flowing the metal around them during the operation of molding. A most characteristic or common form of particle inlaid cast metal surface is the common abrasive inlaid cast metal safety floor and stair tread. This invention has to do specifically with methods for the manufacture of such objects which permit of economically securing control over the distribution of the inlay-particles in the metal surface and of securing a firm bond between the particles and the metal.

In the present art of forming particle inlaid cast metal surfaces, many methods are followed. For instance: A mold may be prepared and the inlay-particles may be sprinkled therein, the pattern returned to the mold and tamped to force the inlay-particles into the mold surface, after which the pattern is removed, the mold closed and the metal poured. Another method is the sprinkling of a powdered refractory material, such as fire clay on the face of the mold, followed by sprinkling the inlay-particles on the fire clay, after which the mold is closed and the metal poured. Or the inlay-particles may be coated with an adhesive composition, such as sodium silicate, and sprinkled into the mold, and after the adhesive is dried by any of several means, the mold may be closed and the metal poured. Another process involves the coating of the mold face with adhesive and sprinkling the inlay-particles thereon. Attempts have been made to use inlay-particles coated with very finely divided metallic particles to secure a bond to the metal, and various other methods have been used. I have observed that in all of these methods there is some tendency for the inlay-particles to be displaced when metal is poured into the mold, and in many of them it is quite marked. In many of these processes for one reason or another, the inlay-particles are quite imperfectly imbedded in and/or bonded to the metal.

This art, as well as the present invention, is also applicable not only to processes for inlaying the surfaces of cast material with abrasives, but for the inlaying of a cast metal surface with particles of any nature such as with other metals, or corrosion resistant particles of any nature, or other related arts, and while the discussion of the present disclosure is directed largely to the production of abrasive inlaid wearing sur-

faces, it is not limited thereto, but is understood to be applicable to analogous arts and the description given is understood to be exemplary thereof.

This invention has for its object the provision of a method of inlaying particles in a cast metal surface whereby control of the final distribution of the particles over the surface is more easily obtained. It has for another important object the provision of a method of inlaying whereby a firmer bonding of the inlaid particles to the metal may be had. It has for an object the provision of a process whereby the surface of such products may be freed to a great degree from the presence of slag, oxide films and the like. It has other objects and advantages which will be in part obvious and part of which will be pointed out hereafter.

It has been observed that in the casting of thin metal sections, as the metal flows over the mold surface, it does not behave as would a liquid which wetted the mold but behaves somewhat as does mercury flowing over a surface which it does not wet, in that a slight skin or film of impurities, oxides and/or colder metal forms on the surface of the metal, and as the metal flows, this skin is rolled under the advancing wave of metal and deposited between the more fluid metal and the mold surface somewhat as a carpet. Due to this, it may be seen that the advancing metal is not capable of flowing freely into interstices as would a limpid liquid, but acts somewhat more in the fashion of a blunt and soft scraper and will to a great extent tend to push before it small particles in its path, rather than to immediately surround them. It is my belief that this behavior of flowing metal in a mold is responsible for many of the difficulties encountered in obtaining uniform or controlled distribution of inlaid particles, since a flow of this sort would tend somewhat to break the bond (however it is arrived at) by which the inlaid particles are held to the surface of the mold and then would tend to displace them, or if the inlaid particles are of lower specific gravity, then, being loosened, they might later rise into the molten metal and so escape from the surface where their presence is desired. It is my belief that this formation of a skin or film of slag impurities or oxides or colder metal separately or in combination, or whatever it may be, also is a major underlying cause that prevents the securing of a good bond between the inlaid particles and the metal. If the skin be slag or oxide, it will persist between the body of the

metal and the inlaid particles, and prevent a good bond. If it merely be colder metal, it will be more viscous and so will not flow freely into the interstices by the inlaid particles and so 5 will not completely surround and imbed them in metal. If the skin be a combination of impurities and colder metal, the result will be the same, but more pronounced.

I have found that by so arranging my mold as 10 to rupture this skin at frequent and repeated intervals and so maintain conditions wherein unfiltered higher temperature limpid metal repeatedly and rapidly may be liberated and brought in contact with the inlay-particle carrying mold surface, I 15 may secure a more even distribution of the inlaid material and a more perfect bonding of the inlaid material with the metal. My method consists of using a mold in which obstructions of a character and distribution designed to secure this 20 repeated film rupture are placed so that the advancing wave of metal will contact them, and of distributing the inlay-particles in the mold with such respect to these obstructions that the benefits of the film rupture may be best secured. For 25 the purposes of the present description, I will refer to these obstructions as dams. It is my belief that as the advancing flow of metal encounters and rises over each of these dams, it is piled up to some slight extent and this piling 30 forces a breaking of the skin formed around the metal and permits hotter, less viscous, and cleaner metal to flow from the interior of the advancing body of metal to surround the inlay-particles just in advance of the point of rupture of the film. 35 It is my belief that a greater portion of the advantages and objects of this invention are attained by this action, although I also believe that the presence of the dams tends to break up the sweep or flow of metal and cut down the velocity 40 of that portion of it adjacent the inlay-particle carrying mold surface, and that this also contributes a portion of the results noted.

What I have found is that in the production of a particle inlaid surface, if the mold be formed 45 so that it presents dams or obstructions to the flow of metal, if these obstructions be reasonably continuous, if they be placed generally transverse to the direction of flow of metal when casting, if the proportions between the height of obstruction and spacing between obstructions be proper, and if inlay-particles be placed on the mold surface between such obstructions, then the various 50 objects and advantages mentioned herein may be obtained.

55 In order to illustrate this invention, I now make reference to a drawing which is attached to and forms a part of this specification. The single figure of this drawing represents a diagrammatic section of a mold with metal flowing thereinto, in 60 which 1 represents the mold, 2 represents the grains of inlaid material on the surface thereof, and 3 represents the dams. 4 is intended to represent the metal flowing into the mold and 5 is intended to represent the film or skin of oxide, or 65 slag-like impurities or of colder metal of which I have spoken above. It will be noted that the direction of flow is assumed to be from left to right and that the dams are placed in a direction transverse to that of the flow of metal. It will be 70 observed that in mounting the dam 3 next the left-hand end, that the metal has piled up behind the dam to an extent which has enabled the hotter metal from the interior to break through the skin and to flow over the dam into the succeeding 75 pocket and surround the inlaid material

therein with a metal which is generally free from this film or skin and which is considerably hotter (possibly 200°-500° F.) than the metal which would normally have been brought in contact with this inlaid material had the film remained unbroken. It will also be observed that adjacent the next dam 3 the film is again forming over the surface of the advancing metal and it must again be broken in order that the hot metal from the interior of the flow may be released to come in 10 contact with the inlaid material to the right of this second dam 3. It will also be observed that these dams are so positioned as to break up and lessen the velocity of sheet flow of the metal over the surface of the mold.

15 The dimensions and spacing of the dams or of the dam forming grooves in the pattern are of importance. I have found that the minimum dimensions of groove to obtain this beneficial result are determined by the following considerations. The depth of groove should preferably be not less than  $\frac{1}{8}$ ", as the beneficial results disappear quite rapidly below this depth. A greater depth of groove will not give increases in protection corresponding to the increases in depth of 20 groove; and too great a depth of groove, say of the nature of  $\frac{1}{2}$ " gives rise to a cascade action of metal on the down stream side, which may displace the inlaid material. As for width, the width 25 of the groove in the pattern or the width of the 30 dam in the mold need only be enough to give the dam sufficient strength to withstand the impact of the flowing metal. I have found for example, that with a groove  $\frac{1}{8}$ " deep, a preferable width 35 is about  $\frac{1}{8}$ ". The proper spacing of the grooves 40 or dams is of special importance. This depends to some extent upon the depth of metal above the dam, that is upon the thickness of the final casting, since in thin sections, the amount of 45 highly heated metal which may flow from the interior of the advancing body after rupture of the film is much less than with thicker sections, and the exact spacing of the grooves depends therefore upon the thickness of the casting to be made. I have found for instance, that on castings only 45  $\frac{1}{16}$ " thick, that the spacing between grooves should not be in excess of approximately  $\frac{3}{4}$ ", while on castings  $1\frac{1}{2}$ " thick, or in excess of that thickness, a spacing of the grooves  $1\frac{1}{2}$ " apart 50 gives rise to good results. For castings of thicknesses between these limits, proportional changes should be made in the spacing of the grooves.

55 With respect to the disposition and general configuration of the dams, the following may be noted. The dams may be continuous or discontinuous, but if discontinuous should not be so short in length that the film is merely punctured by the individual short dam instead of broken for some little space. The dams should be so placed on the mold surface that they are in general transverse to the direction of flow of the 60 entering metal. They may well be disposed in intersecting or interlaced groups to form a pattern in the surface of the final product. Heretofore, I have spoken of the dams as being composed of mold material, and resulting in a groove 65 in the final molded surface. I am not restricted thereto, but find myself able to use and contemplate the use of dams in the mold, which dams are themselves composed of metal or other material, 70 alike or different from the casting body metal and from the inlay-particle material and which, when the operation of casting is finished, will themselves appear in the form of an inlay in the cast surface.

It is to be noted that I may place my inlay-particles in any predetermined location, and affix them there by any of the methods herein discussed. For example; if I am making a stair 5 tread with abrasive inlay, I may place large quantities of abrasive near the front edge, for wear resistance as well as friction, and only place enough in the rest of the tread for friction purposes, and may be assured that the distribution 10 in the final product will be as planned.

I claim:

1. The method of manufacturing articles having particle-inlaid cast metallic surfaces which comprises the steps of providing a mold having 15 a surface on which the inlay-particles are distributed, admitting molten metal to such mold to flow over said mold surface, and while said metal is flowing, repeatedly interrupting the flow and rupturing the film formed over the advancing 20 body of metal to permit portions from the interior thereof to flow forth and surround the inlay-particles adjacent the advancing metal.
2. The method of manufacturing particle-inlaid cast metallic surfaces comprising admitting

molten metal to a mold to flow over and be formed by a surface upon which inlay particles are distributed, said mold surface being additionally provided with obstructions so distributed as to prevent flow along the surface in any direction 5 for any substantial distance and of such size as to cause the metal which overflows the obstruction to come preponderantly from within the obstructed body of flowing metal.

3. The method of claim 2 in which the obstructions are in the form of molded dams from  $\frac{1}{8}$ " to  $\frac{1}{2}$ " in height and spaced from  $\frac{3}{4}$ " to  $1\frac{1}{2}$ " apart.

4. The method of claim 2 in which the obstructions are molded dams disposed in interlacing patterns upon the surface of the mold.

5. The method of claim 2 in which the obstructions are themselves an inlay material and upon cooling of the casting remain in the surface thereof as an inlay, with particles of additional inlay distributed in other portions of the 20 surface.

CARLISLE S. GLEZEN.